



US007553010B2

(12) **United States Patent**  
Pan et al.

(10) **Patent No.:** US 7,553,010 B2  
(45) **Date of Patent:** \*Jun. 30, 2009

(54) **PHASE CHANGE INK IMAGING  
COMPONENT HAVING ELASTOMER OUTER  
LAYER**

(75) Inventors: **David H. Pan**, Rochester, NY (US); **Santokh S. Badesha**, Pittsford, NY (US); **Xiaoying Elizabeth Yuan**, Fairport, NY (US); **Donald S. Stanton**, Penfield, NY (US); **Robert N. Finsterwalder**, Webster, NY (US); **Anthony Yeznach**, Clackamas, OR (US); **Trevor J Snyder**, Newberg, OR (US)

(73) Assignee: **Xerox Corporation**, Norwalk, CT (US)

(\*) Notice: Subject to any disclaimer, the term of this patent is extended or adjusted under 35 U.S.C. 154(b) by 116 days.

This patent is subject to a terminal disclaimer.

(21) Appl. No.: 11/712,637

(22) Filed: Feb. 28, 2007

(65) **Prior Publication Data**

US 2007/0159518 A1 Jul. 12, 2007

**Related U.S. Application Data**

(63) Continuation of application No. 10/920,490, filed on Aug. 17, 2004, now Pat. No. 7,222,954.

(51) **Int. Cl.**  
**B41J 2/01** (2006.01)  
(52) **U.S. Cl.** ..... 347/103; 347/101; 347/102  
(58) **Field of Classification Search** ..... 347/101, 347/103  
See application file for complete search history.

(56) **References Cited**

**U.S. PATENT DOCUMENTS**

|                |         |                 |       |         |
|----------------|---------|-----------------|-------|---------|
| 4,257,699 A    | 3/1981  | Lentz           | ..... | 399/324 |
| 5,166,031 A    | 11/1992 | Badesha et al.  | ..... | 430/124 |
| 5,373,852 A    | 12/1994 | Harrison et al. | ..... | 128/733 |
| 5,736,250 A    | 4/1998  | Heeks et al.    | ..... | 428/447 |
| 6,295,434 B1   | 9/2001  | Chang et al.    | ..... | 399/297 |
| 7,222,954 B2 * | 5/2007  | Pan et al.      | ..... | 347/103 |

\* cited by examiner

*Primary Examiner*—Stephen D Meier

*Assistant Examiner*—Ly T Tran

(74) *Attorney, Agent, or Firm*—Pillsbury Winthrop Shaw Pittman LLP

(57) **ABSTRACT**

An offset printing apparatus having a coated imaging member for use with phase-change inks, has a substrate, an optional intermediate layer, and thereover an outer coating having an elastomer of monomers selected from the group consisting of halogenated monomers, polyorganosiloxane monomers, and mixtures thereof, and an optional heating member associated with the offset printing apparatus.

**19 Claims, 2 Drawing Sheets**



**FIG. 1****FIG. 2**

**FIG. 3**

**PHASE CHANGE INK IMAGING  
COMPONENT HAVING ELASTOMER OUTER  
LAYER**

**CROSS-REFERENCE TO RELATED  
APPLICATIONS**

This is a continuation of U.S. application Ser. No. 10/920, 490 filed Aug. 17, 2004 now U.S. Pat. No. 7,222,954 by the same inventors, and claims priority therefrom. Reference is made to the following commonly assigned, copending patent applications, including U.S. Pat. No. 6,910,765, issued Jun. 28, 2005 entitled, "Phase Change Ink Imaging Component with Outer Layer Having Haloelastomer with Pendant Chains;" U.S. patent application Ser. No. 10/177,780, filed Jun. 20, 2002, entitled, "Phase Change Ink Imaging Component with Thermoplastic Layer;" U.S. patent application Ser. No. 10/177,911, filed Jun. 20, 2002, entitled, "Phase Change Ink Imaging Component With Thermoset Layer;" U.S. patent application Ser. No. 10/177,800, filed Jun. 20, 2002 entitled, "Phase Change Ink Imaging Component with Fluorosilicone Layer;" U.S. Pat. No. 6,918,664, issued Jul. 19, 2005 entitled, "Phase Change Ink Imaging Component with Latex Fluoroelastomer Layer;" U.S. Pat. No. 6,843,559, issued Jan. 18, 2005 entitled, "Phase Change Ink Imaging Component with Mica-Type Silicate Layer;" U.S. Pat. No. 6,932,470, issued Aug. 23, 2005 entitled, "Phase Change Ink Imaging Component with Q-Resin Layer;" U.S. Pat. No. 6,648,467, issued Nov. 18, 2003, entitled, "Phase Change Ink Imaging Component with Polymer Blend Layer;" and U.S. Pat. No. 6,939, 000, issued Sep. 6, 2005 entitled, "Phase Change Ink Imaging Component with Polymer Hybrid Layer." The disclosure of each of these patent applications is hereby incorporated by reference in their entirety.

**BACKGROUND**

The present invention relates generally to an imaging apparatus and layers for components thereof, and for use in offset printing or ink jet printing apparatuses. The layers herein are useful for many purposes including layers for transfer components, including transfix or transfuse components, imaging components, and like components. More specifically, the present invention relates to layers comprising an elastomer and optional filler. In specific embodiments, the elastomer comprises monomers selected from the group consisting of halogenated monomers, polyorganosiloxane monomers, and mixtures thereof. The layers of the present invention may be useful in components used in combination with ink or dye materials. In embodiments, the layers can be used in combination with phase change inks such as solid inks.

Ink jet printing systems using intermediate transfer, transfix or transfuse members are well known, such as that described in U.S. Pat. No. 4,538,156. Generally, the transfix printing or intermediate transfer member is employed in combination with a printhead. A final receiving surface or print medium is brought into contact with the transfix printing surface after the image has been placed thereon by the nozzles of the printhead. The image is then transferred and fixed to a final receiving surface.

More specifically, the phase-change ink transfer printing process begins by first applying a thin liquid, such as, for example, silicone oil, to an imaging member surface. The solid or hot melt ink is placed into a heated reservoir where it is maintained in a liquid state. This highly engineered ink is formulated to meet a number of constraints, including low viscosity at jetting temperatures, specific visco-elastic prop-

erties at component-to-media transfer temperatures, and high durability at room temperatures. Once within the printhead, the liquid ink flows through manifolds to be ejected from microscopic orifices through use of proprietary piezoelectric transducer (PZT) printhead technology. The duration and amplitude of the electrical pulse applied to the PZT is very accurately controlled so that a repeatable and precise pressure pulse can be applied to the ink, resulting in the proper volume, velocity and trajectory of the droplet. Several rows of jets, for example four rows, can be used, each one with a different color. The individual droplets of ink are jetted onto the liquid layer on the imaging member. The imaging member and liquid layer are held at a specified temperature such that the ink hardens to a ductile visco-elastic state.

After depositing the image, a print medium is heated by feeding it through a preheater and into a nip formed between the imaging member and a pressure member, either or both of which can also be heated. A high durometer synthetic pressure member is placed against the imaging member in order to develop a high-pressure nip. As the imaging member rotates, the heated print medium is pulled through the nip and is pressed against the deposited ink image with the help of a pressure member, thereby transferring the ink to the print medium. The pressure member compresses the print medium and ink together, spreads the ink droplets, and fuses the ink droplets to the print medium. Heat from the preheated print medium heats the ink in the nip, making the ink sufficiently soft and tacky to adhere to the print medium. When the print medium leaves the nip, stripper fingers or other like members, peel it from the printer member and direct it into a media exit path.

To optimize image resolution, the transferred ink drops should spread out to cover a predetermined area, but not so much that image resolution is compromised or lost. The ink drops should not melt during the transfer process. To optimize printed image durability, the ink drops should be pressed into the paper with sufficient pressure to prevent their inadvertent removal by abrasion. Finally, image transfer conditions should be such that nearly all the ink drops are transferred from the imaging member to the print medium. Therefore, it is desirable that the imaging member have the ability to transfer the image to the media sufficiently.

The imaging member is multi-functional. First, the ink jet printhead prints images on the imaging member, and thus, it is an imaging member. Second, after the images are printed on the imaging member, they can then transfix or transfuse to a final print medium. Therefore, the imaging member provides a transfix or transfuse function, in addition to an imaging function.

In order to ensure proper transfer and fusing of the ink off the imaging member to the print medium, certain nip temperature, pressure and compliance are required. Unlike laser printer imaging technology in which solid fills are produced by sheets of toner, the solid ink is placed on the imaging member one pixel at a time and the individual pixels must be spread out during the transfix process to achieve a uniform solid fill. Also, the secondary color pixels on the printing member are physically taller than the primary color pixels because the secondary pixels are produced from two primary pixels. Therefore, compliance in the nip is required to conform around the secondary pixels and to allow the primary pixel neighbors to touch the media with enough pressure to spread and transfer. The correct amount of temperature, pressure and compliance is required to produce acceptable image quality.

Currently, the imaging member useful for solid inks or phase change inks comprises anodized aluminum. This mem-

ber operates at about 57° C. to about 64° C. and can be used with a heater that preheats the print media prior to entering the nip. Otherwise, the imaging member may include a heater associated therewith. The heater may be associated anywhere on the offset printing apparatus. The current aluminum imaging member has several drawbacks. A high nip load of up to about 770 pounds is needed for transfix or transfuse operations. Further, because of the high nip load, bulky mechanisms and supporting structures are needed, resulting in increased printer weight and cost. One example is that a fairly complex two-layer pressure roller is needed. In addition, the first copy out time is unacceptable because of the bulky weight. In addition, the first copy out time can be negatively impacted by the bulky weight. Moreover, low cohesive failure temperature is another drawback to use of an anodized aluminum drum.

Several coatings for the imaging member have been suggested. Examples are listed below.

U.S. Pat. No. 5,092,235 discloses a pressure fixing apparatus for ink jet inks having 1) outer shell of rigid, non-compliant material such as steel, or polymer such as acetal homopolymer or Nylon 6/6 and 2) an underlayer of elastomer material having a hardness of about 30 to 60, or about 50 to 60.

U.S. Pat. No. 5,195,430 discloses a pressure fixing apparatus for ink jet inks having 1) outer shell of rigid, non-compliant material such as steel, or polymer such as acetal homopolymer or Nylon 6/6 and 2) an underlayer of elastomer material having a hardness of about 30 to 60, or about 50 to 60, which can be polyurethane (VIBRATHANE, or REN:C: O-thane).

U.S. Pat. No. 5,389,958 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), and a pressure roller with elastomer surface.

U.S. Pat. No. 5,455,604 discloses a fixing mechanism and pressure wheels, wherein the pressure wheels can be comprised of a steel or plastic material such as DELRIN. Image-receiving drum 40 can be a rigid material such as aluminum or stainless steel with a thin shell mounted to the shaft, or plastic.

U.S. Pat. No. 5,502,476 teaches a pressure roller having a metallic core with elastomer coating such as silicones, urethanes, nitrates, or EPDM, and an intermediate transfer member surface of liquid, which can be water, fluorinated oils, glycol, surfactants, mineral oil, silicone oil, functional oils such as mercapto silicone oils or fluorinated silicone oils or the like, or combinations thereof.

U.S. Pat. No. 5,614,933 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and a pressure roller with elastomer surface.

U.S. Pat. No. 5,790,160 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and a pressure roller with elastomer surface.

U.S. Pat. No. 5,805,191 an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and an outer liquid layer of liquid, which can be water, fluorinated oils, glycol, surfactants, mineral oil, silicone oil, functional oils such as 10 mercapto silicone oils or fluorinated silicone oils or the like, or combinations thereof.

U.S. Pat. No. 5,808,645 discloses a transfer roller having a metallic core with elastomer covering of silicone, urethanes, nitriles, EPDM.

15 U.S. Pat. No. 6,196,675 B1 discloses separate image transfer and fusing stations, wherein the fuser roller coatings can be silicones, urethanes, nitrates and EPDM.

U.S. Pat. No. 5,777,650 discloses a pressure roller having an elastomer sleeve, and an outer coating that can be metals, 20 (aluminum, nickel, iron phosphate), elastomers (fluoroelastomers, perfluoroelastomers, silicone rubber, polybutadiene), plastics (polyphenylene sulfide with PTFE filler), thermoplastics (polyethylene, polyamide (nylon), FEP), thermosets (acetals, ceramics). Preferred is anodized aluminum.

25 In addition, many different types of outer coatings for transfer members, fuser members, and intermediate transfer members have been used in the electrostatographic arts using powder toner, but not with liquid inks or phase change inks. Several examples are listed herein.

30 U.S. Pat. No. 5,361,126 discloses an imaging apparatus including a transfer member including a heater and pressure-applying roller, wherein the transfer member includes a fabric substrate and an impurity-absorbent material as a top layer. The impurity-absorbing material can include a rubber elastomer material.

35 U.S. Pat. No. 5,337,129 discloses an intermediate transfer component comprising a substrate and a ceramer or grafted ceramer coating comprised of integral, interpenetrating networks of haloelastomer, silicon oxide, and optionally polyorganosiloxane.

40 U.S. Pat. No. 5,340,679 discloses an intermediate transfer component comprised of a substrate and thereover a coating comprised of a volume grafted elastomer, which is a substantially uniform integral interpenetrating network of a hybrid composition of a fluoroelastomer and a polyorganosiloxane.

45 U.S. Pat. No. 5,480,938 describes a low surface energy material comprising a volume grafted elastomer which is a substantially uniform integral interpenetrating network of a hybrid composition of a fluoroelastomer and a polyorganosiloxane, the volume graft having been formed by dehydrofluorination of fluoroelastomer by a nucleophilic dehydrofluorinating agent, followed by a hydrosilation reaction, addition of a hydrogen functionally terminated polyorganosiloxane and a hydrosilation reaction catalyst.

50 U.S. Pat. No. 5,366,772 describes a fuser member comprising a supporting substrate, and a outer layer comprised of an integral interpenetrating hybrid polymeric network comprised of a haloelastomer, a coupling agent, a functional polyorganosiloxane and a crosslinking agent.

55 U.S. Pat. No. 5,456,987 discloses an intermediate transfer component comprising a substrate and a titamer or grafted titamer coating comprised of integral, interpenetrating networks of haloelastomer, titanium dioxide, and optionally polyorganosiloxane.

60 U.S. Pat. No. 5,848,327 discloses an electrode member positioned near the donor member used in hybrid scavenger-

less development, wherein the electrode members have a composite haloelastomer coating.

U.S. Pat. No. 5,576,818 discloses an intermediate toner transfer component including: (a) an electrically conductive substrate; (b) a conformable and electrically resistive layer comprised of a first polymeric material; and (c) a toner release layer comprised of a second polymeric material selected from the group consisting of a fluorosilicone and a substantially uniform integral interpenetrating network of a hybrid composition of a fluoroelastomer and a polyorganosiloxane, wherein the resistive layer is disposed between the substrate and the release layer.

U.S. Pat. No. 6,035,780 discloses a process for forming a layer on a component of an electrostatographic apparatus, including mixing a first fluoroelastomer and a polymeric siloxane containing free radical reactive functional groups, and forming a second mixture of the resulting product with a mixture of a second fluoroelastomer and a second polysiloxane compound.

U.S. Pat. No. 5,537,194 discloses an intermediate toner transfer member comprising: (a) a substrate; and (b) an outer layer comprised of a haloelastomer having pendant hydrocarbon chains covalently bonded to the backbone of the haloelastomer.

U.S. Pat. No. 5,753,307 discloses fluoroelastomer surfaces and a method for providing a fluoroelastomer surface on a supporting substrate which includes dissolving a fluoroelastomer; adding a dehydrofluorinating agent; adding an amino silane to form a resulting homogeneous fluoroelastomer solution; and subsequently providing at least one layer of the homogeneous fluoroelastomer solution to the supporting substrate.

U.S. Pat. No. 5,840,796 describes polymer nanocomposites including a mica-type layered silicate and a fluoroelastomer, wherein the nanocomposite has a structure selected from the group consisting of an exfoliated structure and an intercalated structure.

U.S. Pat. No. 5,846,643 describes a fuser member for use in an electrostatographic printing machine, wherein the fuser member has at least one layer of an elastomer composition comprising a silicone elastomer and a mica-type layered silicate, the silicone elastomer and mica-type layered silicate form a delaminated nanocomposite with silicone elastomer inserted among the delaminated layers of the mica-type layered silicate.

It is desired to provide a multi-functional imaging member for use with phase change ink printing machines, which has the ability to receive an image, and either transfer or transfer and fuse the image to a print medium. It is desired that the imaging member when having heat associated therewith, be thermally stable for conduction for fusing or fixing. It is further desired that the imaging member have a relatively low nip load, in order to decrease the weight and cost of the printing machine, and in order to provide an acceptable first copy out time.

## SUMMARY

The present invention provides, in embodiments: an offset printing apparatus for transferring a phase change ink onto a print medium comprising: a) a phase change ink component for applying a phase change ink in a phase change ink image; b) an imaging member for accepting the phase change ink image from the phase change ink component, and transferring the phase change ink image from the imaging member to the print medium, the imaging member comprising: i) an imaging substrate, and thereover ii) an outer coating comprising an

elastomer comprising monomers selected from the group consisting of halogenated monomers, polyorganosiloxane monomers, and mixtures thereof.

The present invention further provides, in embodiments: an offset printing apparatus for printing a phase change ink onto a print medium comprising: a) a phase change ink component for applying a phase change ink in a phase change ink image; b) an imaging member for accepting said phase change ink image from said phase change ink component, and transferring the phase change ink image from said imaging member to said print medium and for fixing the phase change ink image to said print medium, the imaging member comprising: i) an imaging substrate, and thereover ii) an outer coating comprising an elastomer comprising monomers selected from the group consisting of halogenated monomers, polyorganosiloxane monomers, and mixtures thereof, and c) a heating member associated with the offset printing apparatus.

In addition, the present invention provides, in embodiments: an offset printing apparatus comprising a phase change ink component containing a phase change ink; a imaging member comprising a substrate, and thereover an outer coating comprising an elastomer comprising monomers selected from the group consisting of halogenated monomers, polyorganosiloxane monomers, and mixtures thereof; and a heating member associated with the offset printing apparatus, wherein the phase change ink component dispenses the phase change ink onto the imaging member, and wherein the phase change ink is solid at room temperature.

## BRIEF DESCRIPTION OF THE DRAWINGS

The above embodiments of the present invention will become apparent as the following description proceeds upon reference to the drawings, which include the following figures:

FIG. 1 is an illustration of an embodiment of the invention, and includes a transfer printing apparatus using an imaging member in the form of a drum.

FIG. 2 is an enlarged view of an embodiment of a transfix printing drum having a substrate and an outer elastomer layer thereon.

FIG. 3 is an enlarged view of an embodiment of a transfix printing drum having a substrate, and optional intermediate layer, and an outer elastomer layer thereon.

## DETAILED DESCRIPTION

The present invention is directed to an offset printing apparatus useful with phase-change inks such as solid inks, and comprising a coated imaging member capable of accepting, transferring and in some embodiments, fixing an ink image to a print medium. The imaging member can be a roller such as a drum, or a film component such as a film, sheet, belt or the like. In embodiments, the imaging member comprises a substrate and an outer layer comprising an elastomer. In an alternative embodiment, the imaging member comprises a substrate, an optional intermediate layer, and outer layer comprising an elastomer. The substrate, intermediate layer, and/or outer layer can further comprise fillers dispersed or contained therein.

The details of embodiments of phase-change ink printing processes are described in the patents referred to above, such as U.S. Pat. Nos. 5,502,476; 5,389,958; and 6,196,675 B1, the disclosures of each of which are hereby incorporated by reference in their entirety.

Referring to FIG. 1, offset printing apparatus 1 is demonstrated to show transfer of an ink image from the imaging

member to a final printing medium or receiving substrate. As the imaging member 3 turns in the direction of arrow 5, a liquid surface 2 is deposited on imaging member 3. The imaging member 3 is depicted in this embodiment as a drum member. However, it should be understood that other embodiments can be used, such as a belt member, film member, sheet member, or the like. The liquid layer 2 is deposited by an applicator 4 that may be positioned at any place, as long as the applicator 4 has the ability to make contact and apply liquid surface 2 to imaging member 3.

The ink used in the printing process can be a phase change ink, such as, for example, a solid ink. The term "phase change ink" means that the ink can change phases, such as a solid ink becoming liquid ink or changing from solid into a more malleable state. Specifically, in embodiments, the ink can be in solid form initially, and then can be changed to a molten state by the application of heat energy. The solid ink may be solid at room temperature, or at about 25° C. The solid ink may possess the ability to melt at relatively high temperatures above from about 85° C. to about 150° C. The ink is melted at a high temperature and then the melted ink 6 is ejected from printhead 7 onto the liquid layer 2 of imaging member 3. The ink is then cooled to an intermediate temperature of from about 20° C. to about 80° C., or about 72° C., and solidifies into a malleable state in which it can then be transferred onto a final receiving substrate 8 or print medium 8.

The ink has a viscosity of from about 5 to about 30 centipoise, or from about 8 to about 20 centipoise, or from about 10 to about 15 centipoise at about 140° C. The surface tension of suitable inks is from about 23 to about 50 dynes/cm. Examples of a suitable inks for use herein include those described in U.S. Pat. Nos. 4,889,560; 5,919,839; 6,174,937; and 6,309,453, the disclosure each of which are hereby incorporated by reference in their entirety.

Some of the liquid layer 2 is transferred to the print medium 8 along with the ink. A typical thickness of transferred liquid is about 100 angstroms to about 100 nanometer, or from about 0.1 to about 200 milligrams, or from about 0.5 to about 50 milligrams, or from about 1 to about 10 milligrams per print medium.

Suitable liquids that may be used as the transfix print liquid surface 2 include water, fluorinated oils, glycol, surfactants, mineral oil, silicone oil, functional oils, and the like, and mixtures thereof. Functional liquids include silicone oils or polydimethylsiloxane oils having mercapto, fluoro, hydride, hydroxy, and the like functionality.

Feed guide(s) 10 and 13 help to feed the print medium 8, such as paper, transparency or the like, into the nip 9 formed between the pressure member 11 (shown as a roller), and imaging member 3. It should be understood that the pressure member can be in the form of a belt, film, sheet, or other form. In embodiments, the print medium 8 is heated prior to entering the nip 9 by heated feed guide 13. When the print medium 8 is passed between the transfix printing medium 3 and the pressure member 11, the melted ink 6 now in a malleable state is transferred from the imaging member 3 onto the print medium 8 in image configuration. The final ink image 12 is spread, flattened, adhered, and fused or fixed to the final print medium 8 as the print medium moves between nip 9. Alternatively, there may be an additional or alternative heater or heaters (not shown) positioned in association with offset printing apparatus 1. In another embodiment, there may be a separate optional fusing station located upstream or downstream of the feed guides.

The pressure exerted at the nip 9 is from about 10 to about 1,000 psi. or about 500 psi, or from about 200 to about 500 psi. This is approximately twice the ink yield strength of

about 250 psi at 50° C. In embodiments, higher temperatures, such as from about 72 to about 75° C. can be used, and at the higher temperatures, the ink is softer. Once the ink is transferred to the final print medium 8, it is cooled to an ambient temperature of from about 20° C. to about 25° C. Stripper fingers (not shown) may be used to assist in removing the print medium 8 having the ink image 12 formed thereon to a final receiving tray (also not shown).

FIG. 2 demonstrates an embodiment of the invention, 10 wherein transfix member 3 comprises substrate 15, having thereover outer coating 16.

FIG. 3 depicts another embodiment of the invention. FIG. 3 depicts a three-layer configuration comprising a substrate 15, intermediate layer 17 positioned on the substrate 15, and outer layer 16 positioned on the intermediate layer 17. In 15 embodiments, an outer liquid layer 2 (as described above) may be present on the outer layer 16.

The imaging member includes an outer layer 16 comprising an elastomer. Examples of elastomers include elastomers 20 comprising halogen monomers, elastomers comprising polyorganosiloxanes, and elastomers comprising halogen monomers and polyorganosiloxane monomers. In one embodiment, the elastomer comprises only halogenated monomers.

Examples of elastomers comprising halogen monomers 25 include fluoroelastomers comprising copolymers and terpolymers of vinylidenefluoride, hexafluoropropylene and tetrafluoroethylene, which are known commercially under various designations as VITON A®, VITON E®, VITON E60C®, VITON E45®, VITON E430®, VITON B 910®, 30 VITON GH®, VITON B50®, VITON E45®, and VITON GF®. The VITON® designation is a Trademark of E.I. DuPont de Nemours, Inc. Three known fluoroelastomers are (1) a class of copolymers of vinylidenefluoride, hexafluoropropylene and tetrafluoroethylene, known commercially as 35 VITON A®, (2) a class of terpolymers of vinylidenefluoride, hexafluoropropylene and tetrafluoroethylene known commercially as VITON B®, and (3) a class of tetrapolymers of vinylidenefluoride, hexafluoropropylene, tetrafluoroethylene and a cure site monomer, for example, VITON® GF. VITON 40 A®, and VITON B®, and other VITON® designations are trademarks of E.I. DuPont de Nemours and Company.

In another embodiment, the fluoroelastomer is a tetrapolymer having a relatively low quantity of vinylidenefluoride. An example is VITON GF®, available from E.I. DuPont de Nemours, Inc. The VITON GF® has 35 weight percent of vinylidenefluoride, 34 weight percent of hexafluoropropylene and 29 weight percent of tetrafluoroethylene with 2 weight percent cure site monomer. The cure site monomer can be those available from DuPont such as 4-bromoperfluorobutene-1, 1,1-dihydro-4-bromoperfluorobutene-1, 3-bromoperfluoropropene-1, 1,1-dihydro-3-bromoperfluoropropene-1, or any other suitable, known, commercially available cure site monomer.

Other fluoroelastomers that may be used include 55 AFLAS®, FLUOREL® I, FLUOREL® II, TECHNOLON® and the like commercially-available elastomers.

Other examples of elastomers include elastomers comprising polyorganosiloxane monomers, and elastomers comprising halogen monomers and polyorganosiloxane monomers, 60 such as polymer composites including, for example, volume grafted elastomers, titamers, grafted titamers, ceramers, and grafted ceramers.

In one embodiment of the invention, the elastomer is a volume grafted elastomer. Volume grafted elastomers are a special form of hydrofluoroelastomer and are substantially uniform integral interpenetrating networks of a hybrid composition of a fluoroelastomer and a polyorganosiloxane, the

volume graft having been formed by dehydrofluorination of fluoroelastomer by a nucleophilic dehydrofluorinating agent, followed by addition polymerization by the addition of an alkene or alkyne functionally terminated polyorganosiloxane and a polymerization initiator.

Volume graft, in embodiments, refers to a substantially uniform integral interpenetrating network of a hybrid composition, wherein both the structure and the composition of the fluoroelastomer and polyorganosiloxane are substantially uniform when taken through different slices of the layer. A volume grafted elastomer is a hybrid composition of fluoroelastomer and polyorganosiloxane formed by dehydrofluorination of fluoroelastomer by nucleophilic dehydrofluorinating agent followed by addition polymerization by the addition of alkene or alkyne functionally terminated polyorganosiloxane. Examples of specific volume graft elastomers are disclosed in U.S. Pat. Nos. 5,166,031; 5,281,506; 5,366,772; and 5,370,931, the disclosures of which are herein incorporated by reference in their entirety.

In embodiments, the polyorganosiloxane has the formula I:



where R is an alkyl from about 1 to about 24 carbons, or an alkenyl from about 2 to about 24 carbons, or a substituted or unsubstituted aryl or heterocyclic of from about 4 to about 24 carbons; A is an aryl or heterocyclic of from about 6 to about 24 carbons, a substituted or unsubstituted alkene of from about 2 to about 8 carbons, such as a vinyl group, a substituted or unsubstituted alkyne of from about 2 to about 8 carbons, or a substituted or unsubstituted alkoxy group having from about 2 to about 8 carbons; and n is from about 2 to about 400, or from about 10 to about 200 in embodiments.

In embodiments, R is an alkyl, alkenyl, aryl or heterocyclic, wherein the alkyl has from about 1 to about 24 carbons, or from about 1 to about 12 carbons; the alkenyl has from about 2 to about 24 carbons, or from about 2 to about 12 carbons; and the aryl or heterocyclic has from about 4 to about 24 carbon atoms, or from about 6 to about 18 carbons. R may be a substituted aryl or heterocyclic group, wherein the aryl or heterocyclic may be substituted with an amino, hydroxy, mercapto or substituted with an alkyl having for example from about 1 to about 24 carbons or from 1 to about 12 carbons, or substituted with an alkenyl having for example from about 2 to about 24 carbons or from about 2 to about 12 carbons. In an embodiment, R is independently selected from methyl, ethyl, and phenyl. The functional group A can be an alkene or alkyne group having from about 2 to about 8 carbon atoms, or from about 2 to about 4 carbons, optionally substituted with an alkyl having for example from about 1 to about 12 carbons, or from about 1 to about 12 carbons, or an aryl or heterocyclic group having for example from about 6 to about 24 carbons, or from about 6 to about 18 carbons. Functional group A can also be mono-, di-, or trialkoxysilane having from about 1 to about 10, or from about 1 to about 6 carbons in each alkoxy group, hydroxy, or halogen. Examples of alkoxy groups include methoxy, ethoxy, and the like. Examples of halogens include chlorine, bromine and fluorine. "A" may also be an alkyne of from about 2 to about 8 carbons, optionally substituted with an alkyl of from about 1 to about 24 carbons or aryl or heterocyclic of from about 6 to about 24

carbons. The group n is from about 2 to about 400, and in embodiments from about 2 to about 350, or from about 5 to about 100. Furthermore, in an embodiment, n is from about 60 to about 80 to provide a sufficient number of reactive groups to graft onto the fluoroelastomer. In the above formula, typical R groups include methyl, ethyl, propyl, octyl, vinyl, allylic crotyl, phenyl, naphthyl and phenanthryl, and typical substituted aryl groups are substituted in the ortho, meta and para positions with lower alkyl groups having from about 1 to about 15 carbon atoms. Typical alkene and alkenyl functional groups include vinyl, acrylic, crotonic and acetyl which may typically be substituted with methyl, propyl, butyl, benzyl, tolyl groups, and the like.

In embodiments, R may be a vinyl group having from about 2 to about 8 carbons, such as  $\text{CH}_2=\text{CHSiR}_2\text{O}(\text{SiR}_2)_n$ —, wherein n is a number of from about 1 to about 100, or from about 1 to about 50, or from about 2 to about 25. In embodiments, R may be an alkoxy group having from about 2 to about 8 carbons, such as  $\text{C}_2\text{H}_5\text{O}—\text{SiR}_2\text{O}—(\text{SiR}_2)_n$ —, wherein n is a number of from about 1 to about 100, or from about 1 to about 50, or from about 2 to about 25. Therefore, the polydimethyl siloxane can be vinyl or alkoxy terminated.

In embodiments, the polyorganosiloxane can be functional poly(dimethylsiloxanes) and silicone resins with auxiliaries such as RT601A Elastosil, or hydrogen-functional dimethylsiloxanes such as RT601B Elastosils from Wacker.

Ceramers are also examples of polymer composites useful as coatings herein. A ceramer generically refers to a hybrid material of organic and composite composition, which typically has ceramic-like properties. As used herein, the term ceramer refers to, in embodiments, a composite polymer comprised of substantially uniform integral interpenetrating networks of a elastomer and silicon oxide. The term grafted ceramer refers to, in embodiments, a composite polymer comprised of substantially uniform integral interpenetrating networks of a polyorganosiloxane grafted haloelastomer and silicon oxide network. In the grafted ceramer, the haloelastomer is the first monomer segment, the polyorganosiloxane is the third monomer segment and the second monomer segment is tetraethoxy orthosilicate, the intermediate to a silicon oxide network. Both the structure and the composition of the polyorganosiloxane grafted haloelastomer and silicon oxide networks are substantially uniform when viewed through different slices of the layer. The phrase interpenetrating network refers to the intertwining of the haloelastomer and silicon oxide network polymer strands for the ceramer, and to the intertwining of the polyorganosiloxane grafted haloelastomer and silicon oxide polymer network strands for the grafted ceramer. The phrase haloelastomer may be any suitable halogen containing elastomer such as a chloroelastomer, a bromoelastomer, or the like, mixtures thereof, and can be a fluoroelastomer. Examples of suitable fluoroelastomers are set forth above. Examples of suitable polyorganosiloxanes are referred to above. The phrases "silicon oxide," "silicon oxide network," "network of silicon oxide" and the like refer to alternating, covalently bound atoms of metal and oxygen, wherein alternating atoms of silicon and oxygen may exist in a linear, branched, and/or lattice pattern. The atoms of silicon and oxygen exist in a network and not as discrete particles. Examples of ceramers and grafted ceramers are described in U.S. Pat. No. 5,337,129, the disclosure of which is hereby incorporated by reference in its entirety.

In an embodiment of the invention, the ceramer has the following formula II:



In the above formula, the symbol “~” represents a continuation of the polymer network.

In an embodiment, a grafted ceramer has the following formula III:



In the above formula, R is the R group of the polyorganosiloxane described above and may be a substituent as defined herein for the R group of the polyorganosiloxane; n is a number as herein defined for the n of the polyorganosiloxane above; and the symbol “~” represents a continuation of the polymer network.

Titamers are also examples of polymer composites suitable for the coatings herein. Titamers are discussed in U.S. Pat. Nos. 5,500,298; 5,500,299; and 5,456,987, the disclosures

each of which are hereby incorporated by reference in their entireties. As used herein, the phrase titamer refers to a composite material comprised of substantially uniform integral interpenetrating networks of haloelastomer and titanium oxide network, wherein both the structure and the composition of the haloelastomer and titanium oxide network, are substantially uniform when viewed through different slices of the coating layer. The phrase grafted titamer refers to a substantially uniform integral interpenetrating networks of a polyorganosiloxane grafted haloelastomer and titanium oxide network, wherein the haloelastomer is the first monomer segment, the polyorganosiloxane is the third grafted monomer segment and titanium isobutoxide, the intermediate to titanium oxide network, is the second monomer segment. Both the structure and the composition of the polyorganosiloxane grafted haloelastomer and titanium oxide network are substantially uniform when viewed through different slices of the coating layer. The phrase “interpenetrating network” refers to the intertwining of the haloelastomer and titanium oxide network polymer strands for the titamer, and to the intertwining of the polyorganosiloxane grafted haloelastomer and titanium oxide network polymer strands for the grafted titamer. The phrase “haloelastomer” may be any suitable halogen containing elastomer such as a chloroelastomer, a bromoelastomer, or the like, mixtures thereof, and can be a fluoroelastomer as described above. The phrase “titanium oxide,” network of titanium oxide,” or “titanium oxide network” or similar phrases refers to alternating, covalently bound atoms of titanium and oxygen, wherein the alternating atoms of titanium and oxygen may exist in a linear, branched and/or lattice pattern. The atom of titanium and oxygen exist in a network and not as discrete particles.

Examples of titamers include those having the following formula IV:



In the above formula, the symbol “~” represents the continuation of the polymeric network.

Examples of grafted titamers include those having the following formula V:



In the above formula, R is the R group of the polyorganosiloxane described above and may be a substituent as defined herein for the R group of the polyorganosiloxane; n is a number as herein defined for the n of the polyorganosiloxane above; and the symbol “~” represents a continuation of the polymer network.

Other examples of suitable elastomers include fluoroelastomers such as fluorourethanes, fluoroacrylate such as LUMIFLON® available from ICI Americas, Inc., Wilmington, Del., and other fluoroelastomers such as polyvinyl fluoride such as TEDLAR®, polyvinylidene fluoride such as KYNAR®, and the like.

In addition, examples of suitable elastomers include those comprising polyorganosiloxane copolymers such as polyamide polyorganosiloxane copolymers, polyimide polyorganosiloxane copolymers, polyester polyorganosiloxane copolymers, polysulfone polyorganosiloxane copolymers, polystyrene polyorganosiloxane copolymers, polypropylene polyorganosiloxane copolymers, and polyester polyorganosiloxane copolymers.

The elastomer is present in the imaging outer layer in an amount of from about 95 to about 35 percent, or from about 90 to about 50 percent, or from about 80 to about 70 percent by weight of total solids. Total solids as used herein refers to the total amount by weight of elastomer, filler, and any additional additives, fillers or like solid materials.

In embodiments, the thickness of the outer imaging layer is from about 0.5 to about 20 mils, or from about 1 to about 6 mils.

The substrate, optional intermediate layer, and/or outer layer, in embodiments, may comprise fillers dispersed therein. These fillers can have the ability to increase the material hardness or modulus into the desired range.

Examples of fillers include fillers such as metals, metal oxides, doped metal oxides, carbon blacks, ceramics, polymers, and the like, and mixtures thereof. Examples of suitable metal oxide fillers include titanium dioxide, tin (II) oxide, aluminum oxide, indium-tin oxide, magnesium oxide, copper oxide, iron oxide, silica or silicon oxide, and the like, and

mixtures thereof. Examples of carbon fillers include carbon black (such as N-990 thermal black, N330 and N110 carbon blacks, and the like), graphite, fluorinated carbon (such as ACCUFLUOR® or CARBOFLUOR®), and the like, and mixtures thereof. Examples of ceramic materials include aluminum nitrate, boron nitride, silicates such as zirconium silicates, and the like, and mixtures thereof. Examples of polymer fillers include polytetrafluoroethylene powder, polypyrrrole, polyacrylonitrile (for example, pyrolyzed polyacrylonitrile), polyaniline, polythiophenes, and the like, and mixtures thereof. The optional filler is present in the substrate, optional intermediate layer, and/or outer layer in an amount of from about 0 to about 30 percent, or from about 1 to about 20 percent by weight of total solids in the layer.

The imaging substrate can comprise any material having suitable strength for use as an imaging member substrate. Examples of suitable materials for the substrate include metals, rubbers, fiberglass composites, and fabrics. Examples of metals include steel, aluminum, nickel, and their alloys, and like metals, and alloys of like metals. The thickness of the substrate can be set appropriate to the type of imaging member employed. In embodiments wherein the substrate is a belt, film, sheet or the like, the thickness can be from about 0.5 to about 500 mils, or from about 1 to about 250 mils. In embodiments wherein the substrate is in the form of a drum, the thickness can be from about  $\frac{1}{32}$  to about 1 inch, or from about  $\frac{1}{16}$  to about  $\frac{5}{8}$  inch.

Examples of suitable imaging substrates include a sheet, a film, a web, a foil, a strip, a coil, a cylinder, a drum, an endless strip, a circular disc, a belt including an endless belt, an endless seamed flexible belt, an endless seamless flexible belt, an endless belt having a puzzle cut seam, a weldable seam, and the like.

In an optional embodiment, an intermediate layer may be positioned between the imaging substrate and the outer layer. Materials suitable for use in the intermediate layer include silicone materials, fluoroelastomers, fluorosilicones, ethylene propylene diene rubbers, and the like, and mixtures thereof. In embodiments, the intermediate layer is conformable and is of a thickness of from about 2 to about 60 mils, or from about 4 to about 25 mils.

Specific embodiments of the invention will now be described in detail. These examples are intended to be illustrative, and the invention is not limited to the materials, conditions, or process parameters set forth in these embodiments. All parts are percentages by weight of total solids as defined above unless otherwise indicated.

## EXAMPLES

### Example 1

#### Preparation of VITON® GF Fluoroelastomer Outer Layer

A fluoroelastomer outer layer was prepared as follows. The overcoating can be comprised of VITON® GF, available from E.I. DuPont and believed to be a fluoropolymer comprised of a tetrapolymer of vinylidene fluoride, hexafluoropropylene, tetrafluoroethylene, and a cure site monomer. A solution of VITON® GF was prepared by dissolving about 500 grams of the GF in about 5 liters of methyl ethyl ketone (MEK) and stirring at room temperature. To approximately 5 liters of this solution, there were added in a reaction vessel 4.4 grams of magnesium oxide, 2.2 grams of calcium hydroxide, 11 grams of E.I. DuPont Curative VC50, and 10 grams of carbon black N991 obtained from Vanderbilt Corporation. The contents of the vessel were ball milled with media for 17 hours.

## 15

The resulting black dispersion containing the VITON® GF can then be spray coated or flow coated to a dry thickness of about 6 mils onto an aluminum imaging substrate.

## Example 2

## Preparation of Volume Graft Fluoroelastomer Outer Layer

A volume graft fluoroelastomer was prepared by dissolving approximately 250 grams of VITON® GF in about 2.5 liters of methylethyl ketone (MEK) by stirring at room temperature. This was accomplished by using a 4 liter plastic bottle and a moving base shaker for about one hour to two hours to accomplish the dissolution. The time needed for dissolving depended upon the speed of the shaker. The above solution was then transferred to a 5 liter Erlenmyer flask and about 25 milliliters of the amine dehydrofluorinating agent, 3-(N-styrylmethyl-2-aminoethyl)aminopropyl trimethoxysilane hydrochloride (S-1590, available from Huls America Inc. Piscataway, N.J.) was added. The contents of the flask were then stirred using a mechanical stirrer while maintaining the temperature between approximately 55 to 60° C. After stirring for about 30 minutes, approximately 50 milliliters of 100 centistoke vinyl terminated polysiloxane (PS-441 also available from Huls America Inc.) was added and stirring was continued for about another ten minutes. A solution of 10 grams of benzoyl peroxide in a 100 milliliter mixture of toluene and MEK (80:20) was then added. The stirring was continued while heating the contents of the flask at about 55° C. for another 2 hours.

During this time, the color of the solution turned light yellow. The solution was then poured into an open tray. The tray was left in the hood overnight (about 16 hours). The resulting yellow rubbery mass left after the evaporation of the solvent was then cut into small pieces with scissors. This material was then extracted extensively and repeatedly with 1,500 milliliters (three 500 milliliter portions) of n-hexane to remove unreacted siloxane. Thereafter, about 54.5 grams of the prepared silicone grafted fluoroelastomer, together with approximately 495 grams of methyl isobutyl ketone, 1.1 grams of magnesium oxide and 0.55 gram of calcium hydroxide ( $\text{Ca(OH)}_2$ ) were added to a jar containing ceramic balls followed by roll milling for 17 to 24 hours until a fine, 3 to 5-micron diameter particle size of the fillers in dispersion was obtained. Subsequently, about 2.5 grams of DuPont CURATIVE VC50 catalyst crosslinker in 22.5 parts of methyl ethyl ketone were added to the above dispersion, shaken for about 15 minutes and the solids content reduced to around 5 to 7 percent by the addition of methyl isobutyl ketone.

Following hand mixing, the mixture can be air sprayed on an imaging substrate to a dry thickness of about 4.5 mils, and cured in ambient dry air for about 24 hours followed by a post step curing procedure involving heating for 2 hours at 93° C., heating for 2 hours at 149° C., heating for 2 hours at 177° C., and thereafter heating for 16 hours at 208° C., followed by cooling.

## Example 3

## Preparation of Volume Graft Outer Layer Using Epoxy Terminated Fluoroelastomer

An aminosilane-coupled polyorganosiloxane fluoroelastomer composition was prepared as follows. A stock solution of VITON® GF obtained from DuPont was prepared by dissolving 250 grams of VITON® GF in 2.5 liters of methylethyl ketone (MEK) with stirring at room temperature for 1 to 2 hours. A four liter plastic bottle and a moving base shaker were used to prepare the stock solution. The above solution

## 16

was then transferred to a four liter Erlenmeyer flask and about 25 ml of the amine dehydrofluorinating agent, N-(2-aminoethyl-3-aminopropyl)-trimethoxysilane (AO700) was added. The contents of the flask were then stirred using a mechanical stirrer while maintaining the temperature between 55 and 60° C. After stirring for about 30 minutes, 12.5 grams of ethoxy terminated polysiloxane (PS 393 available from Huls America Inc.) was added and stirring continued for another 5 minutes. About 25 grams of concentrated aqueous acetic acid catalyst was then added. Stirring was continued while heating the contents of the flask at around 65° C. for another approximate 4 hours. During this time, the color of the solution turned light yellow.

The above yellow solution was then cooled to room temperature. To the solution was added 5 grams of magnesium oxide, 2.5 grams of calcium hydroxide and 12.5 grams of curative VC-50 available from Dow Chemical Co. The above contents were then ball milled with ceramic balls (media) as milling media for around 17 hours. The solution was then diluted to about 5 liters with MEK.

This dispersion can then be spray coated onto an imaging substrate. The substrate can then thermally cured by the following heating procedure: 2 hours at 93° C., 2 hours at 149° C., 2 hours at 177° C., and thereafter heating for 16 hours at 208° C. The thickness of the cured film determined by permascope is expected to be about 4 mils.

## Example 4

## Preparation of Volume Graft Outer Layer Using Hydride Terminated Polysiloxane

An outer layer was prepared as follows. Part A was prepared by dissolving about 500 g of VITON® GF in 5 liters of methylethyl ketone (MEK) by stirring at room temperature as set forth above. The solution was then transferred to a 10 liter Erlenmyer flask and 50 ml of the amine dehydrofluorinating agent, N-(2 aminoethyl)-3-amino propyltrimethoxysilane hydrochloride, available from Huls America Inc. Piscataway, N.J.) was added. The contents of the flask were then stirred using a mechanical stirrer while maintaining the temperature between 55 and 60° C. After stirring for about 30 minutes, 100 ml of 100 centistoke hydride functionally terminated polysiloxane (PS-545, a hydride terminated polydimethyl siloxane plus chloroplatinic acid catalyst, both available from Huls America Inc.) were added and the stirring continued while heating the contents of the flask around 75° C. for another 6 hours. During this time the color of the solution turned light yellow which then was cooled to room temperature. To this solution was then added 10 grams of magnesium oxide, 5 grams of calcium hydroxide and 25 grams of curative VC-50 available from Dow Chemical Co. The above mixture was then ball milled with ceramic balls as media for 17 hours. The mixture was diluted to 12 liters with methylethyl ketone.

A portion of this dispersion (less than 5 liters) can then be spray coated onto an imaging member. The coating can then be air-dried followed by curing using the step heat procedure of Example 3. The thickness of the cured film as determined by permascope is expected to be about 8 mils.

## Example 5

## Preparation of Titamer Outer Layer

To prepare the titamer, a stock solution of VITON® GF was prepared by dissolving about 250 g of VITON® GF in about 2.5 liters of methylethyl ketone (MEK) with stirring at room temperature as set forth in the above examples. The above solution was then transferred to a four liter Erlenmeyer

17

flask and 25 ml of the amine dehydrofluorinating agent, N-2-aminoethyl-3-aminopropyltrimethoxy-silane, (available as A0700 from Huls America Inc.) was added. The contents of the flask were then stirred using a mechanical stirrer while maintaining the temperature as in the above examples. After stirring for about 30 minutes, approximately 62.5 grams of titanium isobutoxide (about 25% by weight based on weight of VITON® GF), available from Huls America Inc., was added and stirring continued for another five minutes. About 25 grams of acetic acid was then added. The stirring was continued while the contents of the flask were heated at around 65° C. for another 4 hours. During this time the color of the solution turned light yellow.

The above yellow solution was then cooled to room temperature. To the above solution was then added 5 grams of magnesium oxide, 2.5 grams of calcium hydroxide and 12.5 grams of E.I. DuPont CURATIVE VC50. The above contents were then ball milled with ceramic balls as media for about 17 hours. The solution was then diluted to about 5 liters with MEK.

This dispersion can then be spray coated on a imaging member to a dry thickness of about 6 mils. The dry titamer film can then be cured by the following heating procedure: 2 hours at 93° C., 2 hours at 149° C., 2 hours at 177° C., and thereafter heating for 16 hours at 208° C. The thickness of the cured titamer film as determined by permascopic is expected to be about 4 mils.

#### Example 6

##### Preparation of Grafted Titamer Outer Layer

A grafted titamer composition was prepared by dissolving about 250 g of VITON® GF in 2.5 liters of methylethyl ketone (MEK) by stirring at room temperature. This was accomplished as set forth in Example 7. The above solution was then transferred to a four liter Erlenmeyer flask and 25 mil of the amine dehydrofluorinating agent, 3-(N-styrylmethyl-2-aminoethylamino)propyltrimethoxysilane hydrochloride (S-1590, available from Huls America Inc.) was added. The contents of the flask were then stirred using a mechanical stirrer while maintaining the temperature between 55 and 60° C. After stirring for about 30 minutes, 50 grams of ethoxy terminated polysiloxane (PS-393) and 50 grams of titanium isobutoxide both available from Huls America Inc. were added and stirring continued for another ten minutes. About 25 grams of acetic acid was then added. The stirring was continued while heating the contents of the flask at around 55° C. for another 4 hours. During this time the color of the solution turned light brown which then cooled to room temperature.

To this solution was then added 5 grams of magnesium oxide, 2.5 grams of calcium hydroxide and 12.5 grams of E.I. DuPont CURATIVE VC50. The above mixture was then ball milled with ceramic balls as media for about 17 hours. The mixture was diluted to 5 liters with methylethyl ketone.

Next, a portion of the above dispersion can be sprayed to a dry thickness of 6.5 mils onto a imaging member. The resulting member can then be cured by the curing profile set forth in Example 7. The member can then cooled to room temperature. The thickness of the cured grafted titamer film as determined by permascopic is expected to be 4.2 mils.

#### Example 7

##### Preparation of Ceramer Outer Layer

A ceramer outer coating was prepared as follows. A stock solution of VITON® GF was prepared by dissolving about

18

250 g of VITON® GF in 2.65 liters of methylethyl ketone (MEK) with stirring at room temperature. A four liter plastic bottle and a moving base shaker were used to prepare the stock solution. The mixture was dissolved for approximately 1 to 2 hours. The above solution was then transferred to a four liter Erlenmeyer flask and about 25 ml of the amine dehydrofluorinating agent, 3-(N-styrylmethyl-2-aminoethylamino)propyltrimethoxysilane hydrochloride (S-1590, available from Huls America Inc.) was added. The contents of the flask were then stirred using a mechanical stirrer while maintaining the temperature between 55 to 60° C. After stirring for about 30 minutes, approximately 12.5 grams of tetraethoxyorthosilicate (TEOS, available from Huls America Inc.) was added and stirring continued for another five minutes. About 25 grams of acetic acid was then added. The stirring was continued while heating the contents of the flask to about 65° C. for another 4 hours. During this time the color of the solution turned light yellow.

The above yellow solution was then cooled to room temperature, and about 5 grams of magnesium oxide, 2.5 grams of calcium hydroxide, and 12.5 grams of E.I. DuPont CURATIVE VC50 were added. The above contents were then ball milled with ceramic balls as media for 17 hours. The solution was then diluted to about 5 liters with MEK.

This dispersion can then be spray coated onto an imaging member to a dry thickness of 4.5 mils. The overcoat can then be cured by using the following heating procedure: 2 hours at 93° C., 2 hours at 149° C., 2 hours at 177° C., and thereafter heating for 16 hours at 208° C. The thickness of the cured film as determined by permascopic is expected to be about 3 mils.

#### Example 8

##### Preparation of a Grafted Ceramer Overcoat

A grafted ceramer composition was prepared by dissolving 250 g of VITON® GF in 2.5 liters of methylethyl ketone (MEK) by stirring at room temperature. This was accomplished by using a four liter plastic bottle and a moving base shaker and dissolving as set forth in Example 7. The above solution was then transferred to a four liter Erlenmeyer flask and about 25 mil of the amine dehydrofluorinating agent, 3-(N-styrylmethyl-2-aminoethylamino)propyltrimethoxysilane hydrochloride (S-1590, available from Huls America Inc.) was added. The contents of the flask were then stirred using a mechanical stirrer while maintaining the temperature between 55 and 60° C. After stirring for about 30 minutes, 50 grams of ethoxy terminated polysiloxane (PS-393) and 50 grams of tetraethoxyorthosilicate both available from Huls America Inc., were added and stirring continued for another ten minutes. About 25 grams of acetic acid was then added. The stirring was continued while heating the contents of the flask at around 55° C. for another 4 hours. During this time, the color of the solution turned light brown which then cooled to room temperature. To this solution was then added 5 grams of magnesium oxide, 2.5 grams of calcium hydroxide and 12.5 grams of E.I. DuPont CURATIVE VC50. The above mixture was then ball milled with ceramic balls as media for 17 hours. The mixture was diluted to 5 liters with methylethyl ketone.

A portion of this dispersion (less than 2 liters) can be spray coated onto an imaging member to a dry thickness of 4.5 mils. The overcoat can be cured by the heating procedure set forth in Example 7. The thickness of the cured film as determined by permascopic is expected to be about 3 mils.

## 19

While the invention has been described in detail with reference to specific embodiments, it will be appreciated that various modifications and variations will be apparent to the artisan. All such modifications and embodiments as may readily occur to one skilled in the art are intended to be within the scope of the appended claims.

What is claimed is:

1. An offset inkjet printing apparatus for transferring a phase change ink onto a print medium comprising:

- a) a phase change ink component for applying a phase change ink in a phase change ink image;
- b) an imaging member for accepting said phase change ink image from said phase change ink component, developing said phase change ink image, and transferring the phase change ink image from said imaging member to said print medium, the imaging member comprising:
  - i) an imaging substrate,
  - ii) an optional intermediate layer, and
  - iii) an outer coating comprising an elastomer comprising monomers selected from the group consisting of halogenated monomers, polyorganosiloxane monomers, and polymers thereof.

2. The offset inkjet printing apparatus of claim 1, wherein an intermediate layer is positioned between said substrate and said outer coating.

3. The offset inkjet printing apparatus of claim 2, wherein said intermediate layer comprises a silicone material.

4. The offset inkjet printing apparatus of claim 3, wherein said intermediate layer comprises a filler.

5. The offset inkjet printing apparatus of claim 4, wherein said filler is selected from the group consisting of carbon blacks, metal oxides, metals, polymers, and mixtures thereof.

6. An offset inkjet printing apparatus of claim 1, wherein said elastomer consists essentially of halogen monomers.

7. The offset inkjet printing apparatus of claim 6, wherein said elastomer is selected from the group consisting of a) copolymers of vinylidenefluoride, hexafluoropropylene, and tetrafluoroethylene, b) terpolymers of vinylidenefluoride, hexafluoropropylene and tetrafluoroethylene, and c) tetrapolymers of vinylidenefluoride, hexafluoropropylene, tetrafluoroethylene, and a cure site monomer.

8. The offset inkjet printing apparatus of claim 1, wherein said elastomer consists essentially of polyorganosiloxane monomers and halogenated monomers.

9. The offset inkjet printing apparatus of claim 8, wherein said elastomer is selected from the group consisting of volume grafted fluoroelastomers, ceramers, grafted ceramers, titamers and grafted titamers.

10. The offset inkjet printing apparatus of claim 1, wherein said elastomer comprises polyorganosiloxane monomers.

## 20

11. The offset inkjet printing apparatus of claim 10, wherein said polyorganosiloxane monomer comprises functionality selected from the group consisting of vinyl, alkoxy and hydrogen functionality.

12. The offset inkjet printing apparatus of claim 10, wherein said elastomer comprises an additional monomer capable of reacting with said polyorganosiloxane monomer to form a polyorganosiloxane copolymer.

13. The offset inkjet printing apparatus of claim 12, wherein said polyorganosiloxane copolymer is selected from the group consisting of polyamide polyorganosiloxane copolymers, polyimide polyorganosiloxane copolymers, polyester polyorganosiloxane copolymers, polysulfone polyorganosiloxane copolymers, polystyrene polyorganosiloxane copolymers, polypropylene polyorganosiloxane copolymers, and polyester polyorganosiloxane copolymers.

14. The offset inkjet printing apparatus of claim 1, wherein said outer coating further comprises a filler.

15. The offset inkjet printing apparatus of claim 14, wherein said filler is selected from the group consisting of metals, metal oxides, carbon blacks, polymers, and mixtures thereof.

16. The offset inkjet printing apparatus of claim 1, wherein said imaging substrate comprises a metal.

17. The offset inkjet printing apparatus of claim 1, wherein said phase change ink is solid at about 25° C.

18. The offset inkjet printing apparatus of claim 1, wherein said phase change ink comprises a dye.

19. An offset inkjet printing apparatus for transferring a phase change ink onto a print medium comprising:

- a) a phase change ink component for applying a phase change ink in a phase change ink image;
- b) an imaging member for accepting said phase change ink image from said phase change ink component, developing said phase change ink image, and transferring the phase change ink image from said imaging member to said print medium, the imaging member comprising:
  - i) an imaging substrate,
  - ii) an optional intermediate layer, and
  - iii) an outer coating comprising a polyorganosiloxane copolymer selected from the group consisting of polyamide polyorganosiloxane copolymers, polyimide polyorganosiloxane copolymers, polyester polyorganosiloxane copolymers, polysulfone polyorganosiloxane copolymers, polystyrene polyorganosiloxane copolymers, polypropylene polyorganosiloxane copolymers, and polyester polyorganosiloxane copolymers.

\* \* \* \* \*